

Patented Nov. 15, 1938

2,136,968

# UNITED STATES PATENT OFFICE

2,136,968

## PHOTOGRAPHIC DEVELOPER

Albert B. Doran, Hollywood, Calif., assignor to  
Carus Chemical Company, Inc., a corporation  
of Illinois

No Drawing. Application October 26, 1936,  
Serial No. 107,736

### 5 Claims. (Cl. 95—88)

This invention relates to an agent for developing light sensitive photographic images and more particularly to a developing agent designed for quick development of silver images in a colloidal medium, particularly gelatin.

Developing agents now available for the quick development of photographic images of the common type are almost entirely combinations of hydroquinone or its derivatives and the corresponding amino benzene derivatives which are known as Metol. Metol is monomethylparaminophenol sulfate. While these products produce rapid development, they have a tendency to cause the development of "graining" in the negative. On the other hand, there are available certain other developers which will produce fine grain but require very long periods of development, for example, as much as twenty-four hours or more.

It has now been discovered that the addition of a halogenated hydroquinone to a salt of a primary aryl amine developer results in the production of fine grain images without resultant decrease in the speed of development. By "benzene type developer" is meant a benzene derivative containing at least two groups selected from the class consisting of hydroxy amino and sulfonic acids and preferably hydroxy or amino.

The addition of minute amounts of a thiocyanate has proved particularly advantageous in connection with such compounds in accelerating the speed of the development without producing enlarged grain size. The amount of thiocyanate must be kept quite low because higher quantities act as silver solvents and adversely affect the films.

Any soluble stable thiocyanate, such as KSCN must be employed, and the compound may be incorporated in quantities ranging from one percent downward, normally to as low as .02%, based on the organic developing agents.

The following is an example of a suitable photographic developer for use on motion picture films.

|                                   |       |      |
|-----------------------------------|-------|------|
| Mono-chloro-hydroquinone          | grams | 1.5  |
| Methyl-ortho-amino-phenol-sulfate | do    | 1.5  |
| Potassium thiocyanate             | do    | .003 |
| Sodium sulfite                    | do    | 80   |
| Hydroquinone                      | do    | 5    |
| Borax                             | do    | 5    |
| Water                             | c. c. | 1000 |

The following example is a suitable formula for fine grain positive development or the development of fine grain plates from a negative, either of sensitized paper, motion picture film, or other light sensitive mediums. Like the preceding formula, it may be modified to suit the requirements of the worker. For developing the

ordinary sensitized paper the solution may be used as shown, or with equal parts of water. For enlarging papers the solution should be diluted with four parts of water. For negative and panchromatic film the solution may be diluted with 4 or 5 parts of water.

|                                   |       |      |
|-----------------------------------|-------|------|
| Mono-chloro-hydroquinone          | grams | 1.5  |
| Methyl-ortho-amino-phenol-sulfate | do    | 1.5  |
| Potassium thiocyanate             | do    | .003 |
| Sodium sulfite                    | do    | 80   |
| Hydroquinone                      | do    | 3    |
| Sodium carbonate                  | do    | 30   |
| Potassium bromide                 | do    | 1    |
| Potassium metabisulfite           | do    | 1    |
| Water                             | c. c. | 1000 |

The following are additional examples of materials which in combination produce suitable developers:

1. A halo-hydroquinone and hydroxymethylparaminophenol sulfate.
2. A chloro-hydroquinone and mono-methylparaminophenol sulfate.
3. A halo-hydroquinone and methyl-ortho-amino-phenol sulfate.
4. A halo-hydroquinone and diphenyl-amino-hydrochloride.

The reason for the effect of the halogenated or thiocyanate compound upon the other developer is not understood. It is possible that the presence of the halogen has some effect upon the release or interchange of halogen radicals upon the silver in the film.

The thiocyanate is effective with benzene type developers in general.

The foregoing detailed description has been given for clearness of understanding only and no unnecessary limitations should be understood therefrom, but the appended claims should be construed as broadly as permissible in view of the prior art.

I claim:

1. A photographic developer comprising approximately equal proportions of mono-chloro-hydroquinone, methyl-ortho-amino-phenol sulfate and .02 to 1 percent of a thiocyanate based on the total weight of the developers.
2. A photographic developer having substantially the following formula:

|                                           |       |      |
|-------------------------------------------|-------|------|
| Mono-chloro-hydroquinone                  | grams | 1.5  |
| Methyl - ortho - amino - phenol - sulfate | grams | 1.5  |
| Potassium thiocyanate                     | do    | .003 |
| Sodium sulfite                            | do    | 80   |
| Hydroquinone                              | do    | 5    |
| Borax                                     | do    | 5    |
| Water                                     | c. c. | 1000 |

3. A photographic developer having substantially the following formula:

|                                           |       |      |
|-------------------------------------------|-------|------|
| Mono-chloro-hydroquinone                  | grams | 1.5  |
| Methyl - ortho - amino - phenol - sulfate | grams | 1.5  |
| 5 Potassium thiocyanate                   | do    | .003 |
| Sodium sulfite                            | do    | 80   |
| Hydroquinone                              | do    | 3    |
| 10 Sodium carbonate                       | do    | 30   |
| Potassium bromide                         | do    | 1    |
| Potassium metabisulfite                   | do    | 1    |
| Water                                     | c. c. | 1000 |

4. A rapidly acting photographic developer comprising a salt of a primary aryl amine developer, a halogenated hydroquinone and a thiocyanate, the thiocyanate being present in amount from approximately .02% to 1%, based on the 5 organic developers present.

5. A developer as set forth in claim 4 in which the thiocyanate is potassium thiocyanate.

ALBERT B. DORAN. 10